

# United States Patent

Kingsbury et al.

[15] 3,652,344

[45] Mar. 28, 1972

[54] **ALUMINUM ALLOY-STEEL BEARING  
AND METHOD OF MAKING SAME**

[72] Inventors: **George R. Kingsbury**, Cleveland;  
**Raymond L. Slater**, Novelty, both of Ohio

[73] Assignee: **Clevite Corporation**

[22] Filed: **Sept. 25, 1969**

[21] Appl. No.: **861,196**

[52] U.S. Cl. .... **148/127, 29/148.4, 29/149.5,**  
**29/196.2, 148/12, 148/12.7, 148/34**

[51] Int. Cl. .... **B21d 53/10, C21d 1/46, C21d 9/40**

[58] Field of Search. .... **148/12, 12.7, 127, 15, 18,**  
**148/34, 159; 29/196.2, 148.4, 149.5**

[56] **References Cited**

UNITED STATES PATENTS

3,268,369 8/1966 Haugen..... 29/196.2 X  
2,807,540 9/1957 Schluchter..... 75/142

3,300,838 1/1967 Slater et al..... 29/196.2 X

OTHER PUBLICATIONS

Metals Handbook, Vol. 2, 8th Ed., 1964, pages 64- 66

Primary Examiner—Charles N. Lovell

Attorney—Eber J. Hyde

[57] **ABSTRACT**

Bimetallic bearing material comprising aluminum alloys consisting of silicon, cadmium, copper, magnesium, and the balance aluminum, bonded directly on steel backings, are heat treated to effect improved hardness and fatigue resistance. The heat treatment comprises solution heating said bearing material at temperatures ranging from 900° F. to 975° F. for at least 15 seconds but not exceeding 80 seconds, after which it is rapidly quenched in a fluid medium having a maximum temperature of 100° F., followed by precipitation heat treatment at about 350° F. for ten hours.

6 Claims, No Drawings

## ALUMINUM ALLOY-STEEL BEARING AND METHOD OF MAKING SAME

The present invention relates to a bearing comprising aluminum alloy directly bonded on a steel backing. More specifically, the invention is concerned with heat treating the bearing material to provide improved fatigue resistance and strength to the finished bearings.

To be acceptable for use in diesel and gasoline engines, bearings of sleeve or flange type must be able to withstand rather high loadings and speeds and be resistant to fatigue and corrosion, in addition to being inexpensive.

The present invention contemplates the method of making bearings comprising aluminum alloys directly bonded onto steel supports or backings. The aluminum alloy consists of aluminum having small amounts of silicon, cadmium, copper, and magnesium. The steel backing can be any of a number of low carbon steels.

Several methods for improving strength and fatigue resistance are disclosed in the prior art. Of note is the method disclosed in U.S. Pat. No. 3,268,369 which teaches, among other things, the step of heating the finished bearing in a nonoxidizing atmosphere at temperatures ranging from 750° F. to just below the eutectic melting point of the aluminum alloy. The above-mentioned patent further teaches that the heating period can be as short as five minutes, but can be longer.

It has been found that solution heat treatments in the order of five minutes and longer are not necessary. In fact, solution heat treatment in the order of 15 seconds is quite satisfactory for obtaining the desired properties of fatigue resistance and strength. Furthermore, heat treatment of finished bearings may be undesirable because of damage to the finely finished bearing surfaces.

It is an object of this invention to provide a bimetallic strip of bearing material and the method of making same, from which low cost, strong, and fatigue resistant bearings are made.

Another object of the invention is to provide a heat treatment for bearing material, in strip, blank, or semifinished bearing form, thereby improving the strength and fatigue resistance of the finished bearings.

A further object of the invention is to provide high quality bearings suitable for use under high loadings and speed conditions.

Other objects and advantages will become more apparent from the following description.

In carrying out the process of the invention, steel of the type commercially known as SAE 1010 or 1008 may be used as the material for the backing support, though other steel types may be used. Low carbon steel is preferred because it endures a greater rolling reduction which results in an improved bond. Also, it has lower initial hardness and is less subject to cold working during cladding and forming.

As to the aluminum alloy, it is directly bonded onto the steel backing to form the bearing material in accordance with the method disclosed in U.S. Pat. No. 3,300,838, assigned to the same assignee of the present invention. The heat-treatment response of the aluminum alloy is related to the copper and magnesium content, as well as the silicon content. Aluminum alloys having silicon 2-8 percent, cadmium 0.5-4 percent, copper 0.05-15 percent, magnesium 0.1-0.2 percent, and the balance aluminum, have proven very satisfactory and the invention contemplates only alloys having the above compositions. The thickness of the layer of aluminum alloy and/or the overall thickness of the composite structure, i.e., the bearing material, depend on the intended use of the finished bearing.

The bimetallic bearing material can be treated in strip, blank, or semi-finished bearing form. When applied to the strip form, the steel backed clad aluminum strip is attached to a pulling unit leading into a molten lead bath maintained at temperature ranging from 900° to 975° F., preferably about 950° F. The strip is then pulled out at a speed permitting it to be heated at said temperature range for a minimum time of 15

seconds. Heat-up time takes usually about a minute. Thus, total immersion in the lead bath may take about 80 seconds. As the strip is being pulled out of the lead bath it is wiped to remove lead particles that may have occluded onto the surface. The strip is then quickly quenched in a fluid medium such as water or oil having a maximum temperature of 100° F., preferably about 75° F. The time between removal from the lead bath to quenching should be such that the temperature of the strip is not allowed to drop below 850° F. Intervals in the order of 30 seconds are usually satisfactory. It should be emphasized that the drop in temperature prior to quenching is of important consideration. The short heating cycle is sufficient to cause the copper, magnesium, and a portion of the silicon to go into solid solution with the aluminum under equilibrium conditions and rapid quenching is necessary to preserve a condition of super saturation.

After quenching, the strip is air dried and hardened by precipitation heat treatment at 350° F. for about ten hours in a recirculating air furnace, or other heating means. A minimum hardness of 62 on the Rockwell 15 T-scale is obtained for 0.010 inch thick aluminum alloy liner. The strip is then fabricated into bearings and the bearing surface is machined and plated at the bearing surface with an overlay having thickness of 0.0004 to 0.0006 inches. The overlay comprises generally a high lead alloy having copper and tin.

The above description alluded to a method of making and heat-treating simple sleeve bearings. If flange bearings are desired, then the bimetallic strip may be heat treated in the molten lead bath as described above. After quenching, the bearing strip is cut into bearing blanks which are channelled, and roll-formed into shells. The formed bearings are then hardened by precipitation heat treatment in a recirculating air furnace at about 350° F. for 10 hours to a minimum R<sub>15</sub> T 62 hardness for a 0.010 inch thick alloy liner.

Other media for solution heat treatment can be utilized such as molten salt baths. For example, the bimetallic strip can be cut into bearing blanks which are then placed in convenient means such as metal baskets which can be lowered into the molten salt bath having a temperature ranging from 900°-975° F. The blanks are then maintained at said temperature for a minimum of 15 seconds excluding heat-up time which is usually about one minute. The blanks are then quenched in a fluid medium such as water (maximum temperature - 100° F.). Again, keeping in mind that the interval between removing from the molten salt bath and the quenching is such that the temperature of the blanks does not drop below 850° F. Normally, a delay time of up to 30 seconds is satisfactory. The blanks are then dried and precipitation hardened at about 350° F. for ten hours in a recirculating air furnace. Bearings are then fabricated from the hardened blanks as described hereinbefore. As to flange bearings, the blanks are channelled and rollformed into shells after the solution heat treatment, then they are precipitation hardened at 350° F., as described.

For uniform results, the bimetallic strip is annealed at 650° F. for 30 minutes prior to solution heat treatment.

Given below are some specific examples of making strong and fatigue resistance bearings from blank form utilizing solution heat treatment in molten salt bath in accordance with the invention.

### EXAMPLE I. DIESEL ROD BEARING

An aluminum alloy having a composition of 3.94 percent silicon, 1.0 percent cadmium, 0.13 percent copper, 0.14 percent magnesium, and the balance aluminum, was directly bonded onto a steel backing (SAE 1010) having a thickness of 0.085 inches to form a bimetallic strip having a thickness of 0.100 inch. The strip was cut into blanks which were heated in a neutral molten salt bath at 950° F. for 65 seconds, 50 seconds were required for heat-up time. The blanks were then removed from the bath and rapidly quenched in water at 75° F. The blanks were then precipitation hardened by heating in an air recirculating furnace at 350° F. for 10 hours. The alu-

minimum alloy layer was found to have an average hardness of 67 on the Rockwell 15 T scale. The blanks were fabricated into bearings with a 0.095 inch wall thickness. The aluminum alloy liner was found to have an average of 69 on R<sub>15</sub> T scale. The bearings were plated with an alloy of 2.5 percent copper, 10 percent tin, 87.5 percent lead. The plate thickness averaged about 0.0005 inch. Bearings of the same composition, but without solution heat treatment, had an average hardness of 50 on R<sub>15</sub> T scale.

#### EXAMPLE II. DIESEL MAIN BEARING

An aluminum alloy having the composition 3.70 percent silicon, 1.10 percent cadmium, 0.15 percent magnesium, 0.10 percent copper, and the balance aluminum, was directly bonded onto an SAE 1010 steel backing (0.139 inch thick) to form a bimetallic bearing strip of 0.166 inch thickness. The strip was cut into blanks which were solution heat treated in a neutral molten salt bath at 950° F., as done in Example I. After precipitation hardening at 350° F. for 10 hours, the average hardness of the aluminum alloy layer measured 69 on R<sub>15</sub> T scale. The blanks were then fabricated into bearings having 0.156 inch wall thickness. Hardness of the aluminum alloy liner had an average of 70 on R<sub>15</sub> T scale. Similar to Example I, the bearing was plated with an over-lay (0.0005 inch thick) having the same composition.

Bearings having the same composition and thickness, but not solution heat treated, had an average hardness of 48 on R<sub>15</sub> T scale.

#### EXAMPLE III. DIESEL FLANGE MAIN BEARING

An aluminum alloy having the same composition of Example II was directly bonded on an SAE 1010 steel backing (0.089 inch thick) to form a bimetallic bearing strip having 0.119 inch thickness. The strip was cut into blanks which were solution heat-treated, similar to Examples I and II. The quenched blanks were then formed into flange bearing half-shells which were precipitation hardened, as described in the previous examples. The aluminum alloy layer was found to have an average hardness of 69 on R<sub>15</sub> T scale. The formed shells were then machined to a wall thickness of 0.102 inch, after which an over-lay of about 0.0005 inch was plated on the bearing surface.

Bearings having the same composition and thickness, but not solution heat treated, had an average hardness of 49 on R<sub>15</sub> T scale.

While there have been described what are considered to be the preferred embodiments of this invention, it will be obvious to those skilled in the art that various changes and modifications may be made therein without departing from the invention.

What is claimed is:

1. A method for making a bimetallic bearing having improved fatigue resistance and strength which comprises the steps of:
  - a. bonding to a steel backing a layer of aluminum alloy consisting of silicon 2 to 8 percent, cadmium 0.5 to 4 percent, copper 0.05 to 0.15 percent, magnesium 0.1 to 0.2 percent, and the balance aluminum, to form a composite bearing material in strip or blank form;
  - b. heating the bearing material to a temperature of at least 900° F., but not in excess of 975° F.;
  - c. maintaining the bearing material at said temperature for a period of at least 15 seconds but not over 80 sec.;

- d. cooling rapidly the bearing material in a fluid medium having a maximum temperature of 100° F.;
  - e. forming the desired shape of the bearing; and
  - f. heating the bearing at a temperature of about 350° F. for a period of about therefor 10 hours to effect precipitation hardening.
2. The method described in claim 1 in which in step (a) the bearing material is made in strip form, in which in step (b) the bearing material is heated in molten lead bath having a temperature range of from 900° to 975° F. and in which in step (d) the fluid medium is water having a maximum temperature of 100° F.
  3. A method for improving fatigue resistance and strength of a bimetallic bearing which comprises the steps of:
    - a. bonding directly to a steel backing a layer of aluminum alloy consisting of silicon 2 to 8 percent, cadmium 0.5 to 4.0 percent, copper 0.05 to 0.15 percent, magnesium 0.1 to 0.2 percent, and the balance aluminum, to form a composite bearing material in strip or blank form;
    - b. annealing said bearing material at a temperature of about 650° F. for about 30 minutes;
    - c. heating said bearing material to a temperature ranging from 900 to 975° F.;
    - d. maintaining said material at said temperature for at least 15 seconds, but not over 80 seconds;
    - e. cooling rapidly the bearing material in a fluid medium having a maximum temperature of 100° F.;
    - f. heating the bearing material at a temperature of about 350° F. for not over 10 hours to effect precipitation hardening;
    - g. forming the desired shape of the bearing.
  4. The method as described in claim 3 in which in step (a) the bearing material is made in strip form; in which in step (c) the bearing material is heated in a medium selected from the group consisting of molten lead and neutral molten salt, and in which in step (e) the fluid medium is water having a maximum temperature of 100° F.
  5. A method for improving fatigue resistance and strength of a bimetallic bearing which comprises the steps of:
    - a. bonding directly to a low carbon steel backing a layer of aluminum alloy consisting of silicon 2 to 8 percent, cadmium 0.5 to 4.0 percent, copper 0.05 to 0.15 percent, magnesium 0.1 to 0.2 percent, and the balance aluminum, to form a composite bearing material;
    - b. annealing said bearing material at a temperature of about 650° F. for about 30 minutes;
    - c. cutting said annealed bearing material into bearing blanks;
    - d. heating said bearing blanks to a temperature ranging from 900° to 975° F.;
    - e. maintaining said bearing blanks at said temperature for at least 15 seconds, but not over 80 seconds;
    - f. cooling rapidly the bearing blanks in a fluid medium having a maximum temperature of 100° F.;
    - g. cleaning and drying said bearing blanks;
    - h. heating said blanks at a temperature of 350° F. for 10 hours to effect precipitation hardening;
    - i. forming the desired shape of the bearing.
  6. The method as described in claim 5 in which in step (d) the bearing blanks are heated in neutral molten salt bath having a temperature range of from 900° to 975° F., and in which in step (f) the fluid medium is water having a maximum temperature of 100° F.